



US008133353B2

(12) **United States Patent**  
**Blanz et al.**

(10) **Patent No.:** **US 8,133,353 B2**  
(b4) **Date of Patent:** **Mar. 13, 2012**

(54) **CREPED PAPER PRODUCT**

(75) Inventors: **John James Blanz**, Mosinee, WI (US);  
**Thomas Brod**, Mosinee, WI (US);  
**Emerson S. Brooks**, Jay, ME (US)

(73) Assignee: **Wausau Paper Corp.**, Mosinee, WI  
(US)

(\*) Notice: Subject to any disclaimer, the term of this  
patent is extended or adjusted under 35  
U.S.C. 154(b) by 739 days.

(21) Appl. No.: **11/080,346**

(22) Filed: **Mar. 15, 2005**

(65) **Prior Publication Data**

US 2006/0207735 A1 Sep. 21, 2006

(51) **Int. Cl.**

**B31F 1/12** (2006.01)  
**D21H 13/24** (2006.01)  
**D21F 11/00** (2006.01)  
**B32B 7/12** (2006.01)  
**B32B 37/26** (2006.01)

(52) **U.S. Cl.** ..... **162/111**; 162/118; 162/135; 162/146;  
162/169; 428/153; 428/34.2; 428/32.81; 428/343;  
428/352; 428/355 BL; 156/183; 264/282

(58) **Field of Classification Search** ..... 162/109,  
162/111-113, 118, 141, 146, 145, 152, 156,  
162/157.1-157.7, 135-137, 158, 197, 204-207;  
428/152-153, 172, 343, 352, 355 BL, 906,  
428/32.81, 41.8, 202; 156/183; 264/282-283

See application file for complete search history.

(56) **References Cited**

## U.S. PATENT DOCUMENTS

2,941,661 A 6/1960 Picard et al.  
2,954,868 A \* 10/1960 Swedish, Jr. et al. .... 428/153  
2,996,425 A \* 8/1961 Hamilton ..... 162/113

3,026,217 A \* 3/1962 Hechtman et al. .... 162/169  
3,124,558 A \* 3/1964 Stucker et al. .... 428/153  
3,154,430 A \* 10/1964 Goodloe et al. .... 162/168.1  
3,156,581 A \* 11/1964 Miller et al. .... 428/343  
3,489,643 A \* 1/1970 Hoffman ..... 162/157.3  
3,503,495 A \* 3/1970 Gustafson et al. .... 428/153  
3,879,257 A 4/1975 Gentile et al.  
4,529,481 A \* 7/1985 Yoshida et al. .... 162/146  
4,637,859 A \* 1/1987 Trokhan ..... 162/109  
4,654,254 A 3/1987 Gerry et al.  
4,834,838 A 5/1989 Klowak

(Continued)

## FOREIGN PATENT DOCUMENTS

EP 0 411 752 A1 2/1991

(Continued)

*Primary Examiner* — Jose A Fortuna

(74) *Attorney, Agent, or Firm* — Merchant Gould, P.C.

(57) **ABSTRACT**

A creped paper product is provided according to the invention. The creped paper product comprises a result of creping a web of fibers comprising synthetic fibers to provide a creped paper product having a stretch of at least 3% in the machine direction according to TAPPI test T494. The web of fibers can include about 0.5 wt. % to 100 wt. % synthetic fibers based on the total weight of the fibers. In addition, the web of fibers can contain about 0.5 wt. % to about 10 wt. % of synthetic fibers and about 90 wt. % to about 99.5 wt. % of cellulosic fibers. When the web of fiber includes a mixture of synthetic fibers and cellulosic fibers, the creped paper product can be provided having a tear strength in the machine direction according to TAPPI test T494 at least 10% greater than an otherwise identical creped paper product that does not contain synthetic fibers. A method for forming a creped paper product is provided according to the invention.

**22 Claims, 3 Drawing Sheets**



## U.S. PATENT DOCUMENTS

|                |         |                      |         |
|----------------|---------|----------------------|---------|
| 4,849,278 A *  | 7/1989  | Stokes .....         | 428/153 |
| 5,223,092 A    | 6/1993  | Grinnell et al.      |         |
| 5,223,093 A    | 6/1993  | Klowak               |         |
| 5,223,095 A *  | 6/1993  | Kinsley, Jr. .....   | 162/146 |
| 5,318,670 A *  | 6/1994  | Link et al. .....    | 162/206 |
| 5,385,783 A *  | 1/1995  | Patel et al. .....   | 428/353 |
| 5,387,319 A *  | 2/1995  | Mora et al. .....    | 162/146 |
| 5,496,601 A *  | 3/1996  | Schurb .....         | 428/415 |
| 5,674,590 A    | 10/1997 | Anderson et al.      |         |
| 5,688,523 A    | 11/1997 | Garbe et al.         |         |
| 5,690,787 A    | 11/1997 | Hultman et al.       |         |
| 6,048,806 A    | 4/2000  | Deeb et al.          |         |
| 6,146,499 A *  | 11/2000 | Lin et al. .....     | 162/197 |
| 6,187,140 B1   | 2/2001  | Anderson et al.      |         |
| 6,193,838 B1 * | 2/2001  | Oriaran et al. ..... | 162/112 |
| 6,277,241 B1   | 8/2001  | Merker et al.        |         |
| 6,458,244 B1 * | 10/2002 | Wang et al. .....    | 162/146 |
| 6,637,697 B1   | 10/2003 | Wienberg             |         |
| 6,774,063 B2   | 8/2004  | Bouchette et al.     |         |
| 6,808,597 B2   | 10/2004 | Allen                |         |
| 6,827,819 B2   | 12/2004 | Dwiggins et al.      |         |
| 6,828,008 B2   | 12/2004 | Gruber               |         |

|                   |         |                         |         |
|-------------------|---------|-------------------------|---------|
| 6,838,154 B1      | 1/2005  | Varona et al.           |         |
| 7,156,953 B2 *    | 1/2007  | Tirimacco et al. .....  | 162/112 |
| 7,189,308 B2 *    | 3/2007  | Feit et al. .....       | 162/180 |
| 2001/0008180 A1   | 7/2001  | Anderson et al.         |         |
| 2003/0051838 A1 * | 3/2003  | Wang et al. .....       | 162/146 |
| 2004/0115431 A1 * | 6/2004  | Chen et al. .....       | 428/373 |
| 2004/0238135 A1 * | 12/2004 | Edwards et al. .....    | 162/111 |
| 2004/0241435 A1 * | 12/2004 | Grittner et al. .....   | 428/354 |
| 2004/0250969 A1 * | 12/2004 | Luu et al. .....        | 162/123 |
| 2005/0247416 A1 * | 11/2005 | Forry et al. .....      | 162/109 |
| 2005/0258576 A1 * | 11/2005 | Forry et al. .....      | 264/517 |
| 2006/0042767 A1 * | 3/2006  | Bhat et al. .....       | 162/117 |
| 2006/0086472 A1 * | 4/2006  | Hermans et al. .....    | 162/111 |
| 2006/0130988 A1 * | 6/2006  | Hermans et al. .....    | 162/123 |
| 2006/0207735 A1 * | 9/2006  | Blanz et al. .....      | 162/111 |
| 2008/0076696 A1 * | 3/2008  | Uitenbroek et al. ..... | 510/515 |

## FOREIGN PATENT DOCUMENTS

|    |              |         |
|----|--------------|---------|
| EP | 454104 A1 *  | 10/1991 |
| EP | 1703017 A1 * | 9/2006  |
| WO | WO 89/01074  | 2/1989  |

\* cited by examiner





FIG. 2



FIG. 3

## 1

## CREPED PAPER PRODUCT

## FIELD OF THE INVENTION

The invention relates to a creped paper product and a method for manufacturing a creped paper product. In particular, the invention relates to a creped paper product including synthetic fibers for enhanced tear strength.

## BACKGROUND OF THE INVENTION

Tape products provided in roll form, such as masking tape, typically include a base sheet of fibrous materials impregnated with a latex composition, and an adhesive is applied to one side and a release coating applied to the opposite side. The coated product is then wound and slit into rolls. In some applications, it is desirable for tape to be stretchable. For example, it is desirable for masking tapes to be stretchable as it allows it to conform well to curved or irregular surfaces.

Creping is a technique used to impart a degree of stretchability to paper. For an example of creping being used to impart stretchability to masking tape, see U.S. Pat. No. 2,941,661 to Picard et al. Creping typically involves impacting paper against a device, such as a blade, resulting in crinkling and at least partial disruption of inter-fiber bonding.

## BRIEF DESCRIPTION OF THE DRAWINGS

FIG. 1 is a schematic diagram of an exemplary process for manufacturing a creped paper product according to the invention.

FIG. 2 is a schematic diagram of an exemplary process for treating a creped paper product with latex and applying a release coating.

FIG. 3 is a schematic diagram of an exemplary process for applying an adhesive composition to a latex treated creped paper product.

## SUMMARY OF THE INVENTION

A creped paper product is provided according to the invention. The creped paper product comprises a result of creping a web of fibers comprising synthetic fibers to provide a creped paper product having a stretch of at least 3% in the machine direction according to TAPPI test T494. The web of fibers can include a sufficient amount of synthetic fiber to increase tear strength. For example, the web of fibers can include about 0.5 wt. % to 100 wt. % synthetic fibers based on the total weight of the fibers. The remaining fiber component, if present, can include cellulosic fibers. The web of fibers can contain about 0.5 wt. % to about 10 wt. % of synthetic fibers and about 90 wt. % to about 99.5 wt. % of cellulosic fibers. When the web of fiber includes a mixture of synthetic fibers and cellulosic fibers, the creped paper product can be provided having a tear strength in the machine direction according to TAPPI test T494 at least 10% greater than an otherwise identical creped paper product that does not contain synthetic fibers.

A method for forming a creped paper product is provided according to the invention. The method includes creping a web of fibers to provide a creped paper product having a stretch of at least 3% in the machine direction according to TAPPI test T494. The web of fibers can include a sufficient amount of synthetic fiber to increase tear strength. For example, the web of fibers can include about 0.5 wt. % to 100 wt. % synthetic fibers based on the total weight of the fibers. The remaining fiber component, if present, can include cellulosic fibers. In addition, the web of fibers can contain about

## 2

0.5 wt. % to about 10 wt. % of synthetic fibers and about 90 wt. % to about 99.5 wt. % of cellulosic fibers. When the web of fiber includes a mixture of synthetic fibers and cellulosic fibers, the creped paper product can be provided having a tear strength in the machine direction according to TAPPI test T494 at least 10% greater than an otherwise identical creped paper product that does not contain synthetic fibers.

## DETAILED DESCRIPTION

10 Creped paper can be obtained by subjecting a web of fibers to a creping technique or process. In general, creping technique involves impacting the web of fibers to create crinkles or crepe lines. Creping tends to have the general effect of increasing stretch. The creped paper product can be referred to more simply as the "paper product" or the "creped paper."

15 The creped paper product can refer to a single layer structure of a web of fibers that has been creped, or to a laminate containing at least one layer of a web of fibers that have been creped. In the case of a laminate, an additional layer can include, for example, a release layer, an adhesive layer, or a release layer and an adhesive layer. The release layer and the adhesive layer can be provided on opposing sides of the creped paper product so that the creped paper product can 20 form, for example, a tape that can be provided in the form of a roll. The web of fibers can be treated with various paper treatment additives such as a latex.

25 The creped paper product can be used in various applications where it is desired to provide a creped paper product having desired stretch and tear strength properties. An exemplary product formed from a creped paper product includes tape such as masking tape. Masking tapes are often applied over a surface to protect the surface from paints, stains, varnishes, etc. that may be applied near the masking tape. Additional products that may benefit from a creped paper product having desired flexibility and tear strength properties include clothing such as medical garments, carpet seaming tape, sewing tape, and book binding.

30 The phrase "machine direction" in reference to the paper product refers to the lengthwise (continuous) direction of the paper product. The machine direction can be referred to as the continuous direction and is the direction along which the paper product travels as it is manufactured. In the case of a roll of tape, the machine direction or continuous direction refers 35 to the direction along which the tape is rolled or unrolled. The phrase "cross direction" or "transverse direction" is the width or direction perpendicular to the continuous direction, of the paper product. By way of example, for a roll of tape having a width of 1 inch and a length of 100 feet, the machine direction refers to the length of 100 feet and the transverse direction refers to the width of 1 inch. It should be understood that the paper product can be provided with any dimension, as desired.

## Manufacture of the Paper Product

40 Referring to FIG. 1, a process for making a creped paper product according to the invention is shown at reference numeral 10. It should be understood that FIG. 1 is an exemplary schematic diagram and includes many of the operations carried out in commercial paper making facilities. The equipment used in a particular operation may vary from facility to facility and the sequence of many operations performed can be altered. It is expected that many of the same general operations will be present in many facilities for making creped paper.

45 55 60 65 65 A starting material 12 can be referred to as pulp 14 and can be processed through a refining operation 16 and through a cleaning operation 18 to provide cleansed pulp 20. The

cleansed pulp 20 can be applied through a head box 22 onto a papermaking machine 24 such as a fourdrinier machine to create a web of fibers 26. The papermaking machine 24 can create the web of fibers 26 by a wet laid technique. The side of the web of fibers 26 facing down on the papermaking machine 24 can be referred to as the "wire side," and the side of the web of fibers 26 facing up on the papermaking machine 24 can be referred to as the "felt side." Additives added at or before the head box 22 can be referred to as "wet end chemistry." The web of fibers 26 can be processed through a wet press to remove water and to provide an intermediate paper substrate 32. If desired, a dryer can be provided to reduce the water content of the intermediate paper substrate 32.

The intermediate paper substrate 32 can be subjected to creping at a creping press 34. The desired water content of the intermediate paper substrate 32 prior to creping may be selected depending upon the particular creping technique utilized. The intermediate paper substrate 32 can be creped in a wet state or in a dry state. For example, it may be desirable to reduce the water content of the intermediate paper substrate 32 to less than about 80 wt. % prior to creping, and it may be desirable to reduce the water content of the intermediate paper substrate 32 to less than about 60 wt. % prior to creping. One would understand how dryers could be used to reduce water content to a desired level for creping.

Various techniques for creping are available. In general, creping involves the impacting of the intermediate paper substrate 32 against a device, such as a blade, resulting in crinkling and at least a partial disruption of inter-fiber bonding.

The creping can be performed as part of the paper making process ("on machine") or as part of a procedure separate from the paper making process ("off machine"). As shown in FIG. 1, the creping is performed "on machine." The substrate recovered from the creping press 34 can be referred to as the rough creped paper substrate 40. The rough creped paper substrate 40 can be further processed as desired. For example, the rough creped paper substrate 40 can be further dried, treated with a composition such as a latex, or a combination of both. Additives added to a paper substrate using a size press can be referred to as "size press chemistry." It is known that additives can be incorporated into paper using, for example, wet end chemistry, size press chemistry, or a combination of wet end chemistry and size press chemistry.

The rough creped paper 40 having the desired water content can pass through a machine calender 42 to provide a finished creped paper product 50. The finished creped paper product 50 can be referred to as the creped paper product and can be sent to a winder 44 and taken up on a roll 46 as roll stock 48. The finished creped paper product 50 can be sold as roll stock 48 or further processed for additional processing such as that described in FIGS. 2 and 3.

Referring now to FIG. 2, a schematic view of an exemplary process for application of latex and a release coating to a creped paper substrate is shown at reference number 70. The finished creped paper product 50 is taken off the roll stock 48 and treated with a latex composition at a bath 72. Many different latex compositions are known in the art and can be used to treat the creped paper product. The creped paper product 50 can be fed to a dryer 74, such as an air floatation dryer. The creped paper substrate 50 can be fed to a coating station 76 that applies a release layer composition onto one side of the creped paper substrate 50 forming an intermediate tape product 82. Many different release layer compositions are known in the art. An example of a suitable release layer composition is disclosed in U.S. Pat. No. 2,941,661 (Picard et al.). One of skill in the art will appreciate that many different pieces of equipment may be used to apply the release layer

including roll coaters, gate-roll coaters, blade coaters, metering size presses, bill blade coaters, sprayers, and the like. After the release layer is applied, the intermediate tape product 82 can be fed to another dryer 78, such as another air floatation dryer. The dried intermediate tape product 82 can be wound onto a roll 80 as roll stock 81.

Referring now to FIG. 3, a schematic view of an exemplary process for applying an adhesive composition to an intermediate tape product 82 is shown at reference number 90. The intermediate tape product 82 is taken off the roll stock 81 and fed to an adhesive coating station 84. An adhesive layer is applied to the intermediate tape product 82 forming a finished tape product 86. The finished tape product may pass through a dryer (not shown) before continuing on for further processing including slitting and winding and the formation of end user rolls.

It should be understood that FIGS. 2 and 3 are exemplary schematic diagrams and include many of the operations carried out in converting the finished creped paper product 50 into a tape product such as a masking tape. The techniques of FIGS. 2 and 3 can be combined if it is desirable to avoid rolling the intermediate tape product 82 into the roll stock 81. Similarly, the techniques of FIG. 2 or 3 or both can be combined with the technique of FIG. 1 if it is desirable to avoid rolling the finished creped paper product 50 into the roll stock 48.

#### Synthetic Fibers

The Applicants have found that the tear strength of a creped paper product can be increased by the addition of synthetic fiber to the pulp used to form the web of fibers. Incorporating synthetic fibers into a web of fibers can increase the tear strength of creped paper products. The increase in tear strength can be measured in comparison to an otherwise identical creped paper product except not containing the synthetic fiber. Accordingly, the synthetic fiber is provided in the creped paper product in an amount sufficient to increase the tear strength relative to the creped paper product without the synthetic fiber.

The increase in tear strength can be provided for creped paper products that are not latex treated and for creped paper products that are latex treated. In general, latex treatment refers to the application of a latex composition to the web of fibers. A latex composition refers to an aqueous polymer composition that can be provided in the form of an emulsion, a dispersion, or a combination of an emulsion and a dispersion.

The web of fibers can include a sufficient amount of the synthetic fiber so that the dry tear strength of the resulting crepe paper product, as measured in the machine direction according to TAPPI test T414, is greater than an otherwise identical creped paper product that does not contain synthetic fibers. It should be understood that the reference to "an otherwise identical creped paper product that does not contain synthetic fibers" refers to a creped paper product prepared by the same technique except that the web of fibers includes non-synthetic fibers in place of the synthetic fibers. It is generally expected that the non-synthetic fibers will be the same type of fibers as the remaining non-synthetic fibers provided in the web of fibers. The dry tear strength of a creped paper product containing synthetic fibers, as measured in the machine direction according to TAPPI test T414, can be at least 10% greater than an otherwise identical creped paper product that does not contain synthetic fibers. The dry tear strength of a creped paper product containing synthetic fibers, as measured in the machine direction according to TAPPI test T414, can be at least 20% greater than an otherwise identical creped paper product that does not contain synthetic fibers.

This improvement can be seen in both creped paper products that have and have not been treated with a latex composition.

Treating a creped paper product with a latex composition can result in a decrease in dry tear strength. The Applicants have found that incorporating an amount of synthetic fiber into the web of fibers can increase tear strength of a creped paper product formed from a web of fibers that is latex treated. Dry tear strength of a creped paper product treated with a latex, as measured in the machine direction according to TAPPI test T414, can be at least 10% greater than an otherwise identical creped paper product that does not contain synthetic fibers. The increase in tear strength of a creped paper product treated with a latex can be at least about 20%, at least about 30%, and at least about 40% greater than an otherwise identical creped paper product that does not contain the synthetic fiber.

Creped paper containing synthetic fiber as at least part of the web of fibers can have an increase in dry tear strength, as measured in the cross direction according to TAPPI test T414, that is greater than an otherwise identical creped paper product that does not contain the synthetic fiber. The increase in dry tear strength in the cross direction can be at least 10% greater than an otherwise identical creped paper product that does not contain the synthetic fibers. The dry tear strength can be greater than 20%, greater than 30%, and greater than 40% than an otherwise identical creped paper product that does not contain the synthetic fibers. The increase in tear strength in the cross direction can be seen for both creped paper product that does not contain latex treatment and creped paper product that does contain latex treatment.

Various synthetic fibers can be added to a web of fibers to increase tear strength. The synthetic fibers can be selected so that they process desirably in the paper making process. Exemplary synthetic fibers include polyester, polypropylene, polyethylene, polyolefin, rayon, nylon, acrylic, glass, and polyvinyl alcohol. An exemplary synthetic fiber that can be used is polyester. The synthetic fibers can be provided as multicomponent fibers such as bicomponent fibers having different polymers forming part of the same fiber. An exemplary bicomponent fiber includes a core and sheath fiber. An exemplary core and sheath fiber includes a fiber having a polyester core and a polyethylene sheath. Various additional forms of bicomponent fibers include structures that can be characterized as concentric sheath/core, eccentric sheath/core, side-by-side, pie wedge, hollow pie wedge, islands/sea, and three islands. The various forms may provide advantages for particular applications.

The synthetic fiber can be provided in various forms so that the resulting paper product has desired properties. For example, the synthetic fiber can be provided as crimped or non-crimped. Exemplary forms of crimped fiber include spiral crimped, two-dimensional crimped, coil springs, and helical fibers. The fiber can be provided having various cross sectional shapes such as solid round, hollow, trilobal, and ribbon. The various cross sections may provide advantages for particular applications.

The unit "denier" is a measure of mass of fiber per length of fiber. For example, denier is often expressed as grams per 9,000 meters. Denier is often used to characterize the fineness of a fiber. Fibers characterized as having a relatively low denier are generally considered to be fairly fine while fibers characterized as having a higher denier are often referred to as thicker fibers. If the fibers have a denier that is too low, it is expected that the web of fibers may not achieve a desired increase in tear strength. If the denier is too high, it may be difficult for the synthetic fibers to interact and entangle with the web of fibers. The selection of the appropriate denier for

a fiber depends on a number of factors including the chemistry and properties of the polymer. By way of example, it is expected that the synthetic fibers can be provided having a size of at least about 0.1 denier and the synthetic fibers can be provided having a size of less than about 25 denier. In addition, the synthetic fibers can be provided having a size of about 0.5 denier to about 10 denier, and can have a size of about 1 denier to about 5 denier.

The length of the synthetic fiber can be selected to provide 10 the desired level of tear strength increase as a result of the incorporation of the synthetic fiber. If the synthetic fibers have a length that is too small, it is expected that there may not be a desired increase in tear strength. If the synthetic fibers have a length that is too large, it may be difficult to process the 15 synthetic fibers on conventional paper making equipment that utilize a wet laid technique. Longer fibers may be applied using other techniques for forming a non-woven including needle punching, hydroentangling, stitch bonding, or carding. For example, in a wet laid application, the synthetic fibers 20 can have an average length of at least about 1 mm to provide an increase in tear strength, and can be provided having an average length of less than about 8 mm to avoid processing difficulties resulting from the length of the fiber. The synthetic fiber can be provided having an average length of about 2 mm 25 to about 7 mm, and can have an average length of about 3 mm to about 6 mm. If the manufacturing equipment can handle longer fibers, it may be desirable to utilize synthetic fibers having a length of up to about 100 mm. In addition, it may be desirable to utilize synthetic fibers having a length of about 1 30 mm to about 75 mm.

The fibers used to form the web of fibers can contain an amount of synthetic fibers to provide enhanced or increased tear strength compared with an otherwise identical web of fibers but not containing the synthetic fibers. In general, if 35 there is too little amount of synthetic fibers, there may not be a desired increase in tear strength. The amount of synthetic fiber to achieve a desired increase in tear strength may depend on certain properties of the synthetic fiber including denier, length, and the polymer. For example, the web of fibers can 40 contain at least about 0.5 wt. % synthetic fibers, based upon the total weight of the fiber. The amount of synthetic fibers can be at least about 1 wt. % and can be at least about 1.5 wt. %. It is expected that all of the fiber can be provided as 45 synthetic fiber. That is, 100% of the web of fibers can be provided as synthetic fibers. In addition, it is expected that tear strength will increase with the increasing percentage of synthetic fiber. A disadvantage with large amounts of synthetic fiber is the cost associated with the synthetic fiber. Accordingly, it may be desirable from an economic perspective 50 to increase the amount of pulp or cellulosic fiber and decrease the amount of synthetic fiber. The Applicants have found that above levels of synthetic fiber of about 10 wt. %, based on the total weight of the fiber, the increase in tear strength may not be as great. Accordingly, it may be desirable 55 to provide the level of synthetic fiber at less than about 10 wt. %. In addition, it may be desirable to provide the amount of synthetic fiber as less than about 6 wt. % based on the total weight of the fiber. In addition, it may be desirable to provide the synthetic fiber in an amount of about 2 wt. % to about 5 wt. % based on the total weight of the fiber.

#### Creping

One of skill in the art will appreciate that many different methods may be used to crepe paper. An exemplary creping press can include a first crepe press roll made of a soft material and a second crepe press roll made of a more rigid material such as steel. The web of fibers can travel between the rolls and adhere to and follow the second crepe press roll. The

web of fibers can be creped off the second crepe press roll using a doctor blade (or creping blade) to produce a rough creped paper substrate.

The web of fibers that is creped can be characterized as wet or dry. Creping a wet web of fibers can be referred to as wet creping, and creping a dry web of fibers can be referred to as dry creping. In the case of wet creping, it can be desirable for the web of fibers to have a water content of about 20 wt. % to about 65 wt. %. In addition, the web of fibers can have a moisture content of about 35 wt. % to about 60 wt. %. Dry creping is generally characterized as creping a web of fibers having a moisture content of less than about 20 wt. %.

Creping is provided to impart a degree of stretchability to a paper substrate. Stretching properties may be measured according to TAPPI test T494. The web of fibers can be creped to provide a creped paper product having a stretch of at least about 3% in the machine direction (MD) according to TAPPI test T494. Although the web of fibers can be creped to provide a crepe paper product having the desired stretchability, it is generally expected that the stretchability will be less than about 30% in the machine direction (MD) according to TAPPI test T494. The creped paper product can be provided having a stretch of about 3% to about 15% in the machine direction (MD) according to TAPPI test T494, and can be provided having a stretch of about 8% to about 12% in the machine direction according to TAPPI test T494.

The creping process results in the formation of creping lines on the rough creped paper substrate. In general, creped paper having a relatively low number of lines per lineal inch can be associated with heavy papers that are generally more abrasive and rougher compared with creped paper having more crepe lines per lineal inch to produce lighter papers that are finer and smoother. It should be understood that this is just a general characterization and heavy papers can include a higher number of crepe lines per lineal inch than lighter papers. When providing more abrasive and rougher creped paper, the creping process can provide about 5 to about 15 crepe lines per lineal inch. For finer and smoother creped paper products, it may be desirable to provide at least about 15 crepe lines per lineal inch. It is expected that the number of crepe lines can be as large as desired for a particular application. For example, it may be desirable to provide creped paper having in excess of 100 crepe lines per lineal inch. For example, it may be desirable to provide creped paper having up to about 200 crepe lines per lineal inch. For masking tape applications where it is generally desirable to provide a fine and smooth paper product that does not wear and tear on a user's thumb and finger, the creped paper product can include crepe lines of about 15 to about 100 per lineal inch, about 17 to about 50 per lineal inch, and about 20 to about 30 per lineal inch.

#### Wet End Chemistry

Wet end additives can be provided for imparting strength, opacity, color, etc. Exemplary wet strength additives include urea-formaldehyde, melamine-formaldehyde, and polyamide. Exemplary dry strength additives include starches (such as cationic potato starch). One of skill in the art will appreciate that many different types of starches can be used such as corn starch, rice starch, tapioca starch, and wheat starch. Exemplary colorants include dyes, pigments, and opacifying color additives. Exemplary opacifying additives include kaolin clays, titanium dioxide, and calcium carbonate. One of skill in the art will appreciate that these components may be added in many different ways including being added as a part of a batch control process or being added through a metering system for continuous operations. Other components, such as defoaming agents, pitch dispersants,

plasticizers (urea), etc. may also be added prior to the head box. Acid alum (aluminum sulfate and sulfuric acid) may be added prior to the head box. Acid alum can serve various purposes including drainage enhancement, rosin sizing, part of certain retention aid programs, dye fixation, cationic source, acidic buffer. Sizing agents that increase water hold-out are also sometimes added as a part of wet end chemistry.

Bulking agents can be added as a part of wet-end chemistry. However, while not intending to be bound by theory, it is believed that certain types of bulking agents may result in reduced dry tear strength of the finished creped paper product. In an embodiment, the creped paper product of the invention includes less than 14% by weight of bulking agents. In an embodiment, the creped paper product of the invention includes less than 10% by weight of bulking agents. In an embodiment, the creped paper product of the invention includes less than 5% by weight of bulking agents. In an embodiment, the creped paper product of the invention includes about 0.0% by weight of bulking agents.

#### Size Press Chemistry

Size press additives can be provided for sizing, strength, coloring, to close up the surface of the sheet (film formers such as sodium alginate), to fill in the surface of the sheet, for water resistance, and/or oil resistance. Exemplary water resistance additives include alkyl ketene dimer (AKD), styrene maleic anhydride (SMA), and waxes. Exemplary oil resistance additives include fluorocarbons. Exemplary fillers include kaolin clays, titanium dioxide, and calcium carbonate. Plasticizers may also be added at the size press **50**. Plasticizers include humectants and can function to keep paper soft and make it less likely that the paper will fracture. Suitable plasticizers include urea, nitrates, glycerine, and saccharides.

It will be appreciated that there are alternative techniques for applying components to a paper product besides a size press. Other application techniques including roll coaters, gate-roll coaters, blade coaters, metering size presses, bill blade coater, and sprayers may also be used to apply components to the rough creped paper substrate as a part of the paper making machine ("on machine") or as a part of a procedure entirely separate from the paper making machine ("off machine"). By way of example, otherwise finished paper may be unrolled and then fed through a separate machine to apply a specific component.

#### Latexes

Latexes can be applied to a web of fibers to enhance delamination resistance, barrier, or stretch properties. A latex composition can be used to hold the web of fibers together so that the resulting product resists delamination. For various applications of the paper product, it may be desirable to increase the barrier properties or hold out properties. In the case of tape such as masking tape, it is generally desirable that paint, stain, or varnish does not penetrate through the masking tape and discolor the surface beneath the masking tape. Accordingly, a web of fibers may be treated with a latex to increase hold out. In addition, the hold out may be designed for water hold out, organic solvent hold out, or combination of both. The latex treatment may be provided to enhance the stretch of the web of fibers. By applying the latex so that it enters into the web of fibers rather than resting on top of the web of fibers as a coating, it may be possible to help adhere the fibers together to improve the stretch of the web of fibers.

By way of example, suitable latexes include polyacrylates, styrene-butadiene copolymers, styrene-acrylic copolymers, ethylene-vinyl acetate copolymers, nitrile rubbers, polyvinyl chloride, polyvinyl acetate, ethylene-acrylate copolymers, and vinyl acetate-acrylate copolymers. Examples of poly-

acrylates include those sold under the trade names HYCAR® and CARBOSET® available from B.F. Goodrich Company, Cleveland, Ohio, and RHOPLEX® available from Rohm and Haas Company, Philadelphia Pa. Examples of styrene-butadiene copolymers include those sold under the trade names BUTOFAN® available from BASF Corporation, Ontario Canada and DL-219 and DL-283 available from Dow Chemical Company, Midland, Mich. Examples of ethylene-vinyl acetate copolymers include those sold under the trade name DUR-O-SET® available from National Starch and Chemical Co., Bridgewater, N.J. Examples of nitrile rubbers include those sold under the trade name HYCAR® available from B.F. Goodrich Company, Cleveland, Ohio. Examples of polyvinyl chlorides include those sold under the trade name GEON® available from B.F. Goodrich Company, Cleveland, Ohio. Examples of polyvinyl chlorides include those sold under the trade name VINAC® available from Air Products and Chemicals, Inc., Naperville, Ill. Examples of ethylene-acrylate copolymers include those sold under the trade names MICHEM® PRIME available from Michelman, Inc., Cincinnati, Ohio, and ADCOTE® available from Morton Thiokol, Inc., Chicago, Ill. Examples of vinyl acetate-acrylate copolymers include those sold under the trade name XLINK® available from National Starch and Chemical Co., Bridgewater, N.J.

#### Web of Fibers

One of skill in the art will appreciate that the web of fibers can comprise many different types of fibers, both natural and synthetic. Natural fibers from plants can often be referred to as cellulosic fibers. Exemplary natural fibers that can be used include wood fibers and non-wood natural fibers such as vegetable fibers, cotton, various straws (wheat, rye, and others), various canes (bagasse and kenaf), grasses (bamboo, etc.), hemp, corn stalks, etc.

The pulp used for creating the web of fibers can include hardwood fibers, softwood fibers, or a blend of hardwood and softwood fibers. The pulp can be provided as cellulose fiber from chemical pulped wood, and can include a blend from coniferous and deciduous trees. By way of example, the fibers can be from northern hardwood, northern softwood, southern hardwood, or southern softwood. Hardwood fibers tend to be more brittle but are generally more cost effective for use because the yield for pulp from hardwood is higher than the yield for pulp from softwood. The pulp can contain about 0 to about 70% hardwood fibers. Softwood fibers have better paper making characteristics but are more expensive. The pulp can contain about 0 to about 100% softwood fibers. The pulp can contain a blend of hardwood and softwood fibers. In an embodiment, the pulp can contain greater than 70% natural fibers. In an embodiment, the pulp contains greater than 80% natural fibers. In an embodiment, the pulp can contain greater than 90% natural fibers. In an embodiment, the pulp can contain 97% natural fibers and 3% polyester fibers as measured by weight. In an embodiment, the pulp contains 97% northern softwood and 3% polyester fibers as measured by weight.

The natural fibers used in the invention can be extracted with various pulping techniques. For example, mechanical or high yield pulping can be used for stone groundwood, pressurized groundwood, refiner mechanical pulp, and thermo-mechanical pulp. Chemical pulping can be used incorporating kraft, sulfite, and soda processing. Semi-chemical and chemi-mechanical pulping can also be used which includes combinations of mechanical and chemical processes to produce chemi-thermomechanical pulp.

The fibers can also be bleached or unbleached. One of skill in the art will appreciate that the bleaching can be accom-

plished through many methods including the use of chlorine, hypochlorite, chlorine dioxide, oxygen, peroxide, ozone, or a caustic extraction.

The pulp can also include post-consumer waste (PCW) fiber. Post-consumer waste fiber is recovered from paper that is recycled after consumer use. Post-consumer waste fiber can include both natural and synthetic fiber. Incorporation of PCW fiber can aid in efficient use of resources and increase the satisfaction of the end user.

10 Refining is the treatment of pulp fibers to develop their papermaking properties. Refining increases the strength of fiber to fiber bonds by increasing the surface area of the fibers and making the fibers more pliable to conform around each other, which increases the bonding surface area and leads to a denser sheet, with fewer voids. Most strength properties of paper increase with pulp refining, since they rely on fiber to fiber bonding. The tear strength, which depends highly on the strength of the individual fibers, actually decreases with refining. Refining of pulp increases the fibers flexibility and leads 15 to denser paper. This means bulk, opacity, and porosity decrease (densometer values increase) with refining. Fibrillation is a result of refining paper fibers. Fibrillation is the production of rough surfaces on fibers by mechanical and/or chemical action; refiners break the outer layer of fibers, i.e., 20 the primary cell wall, causing the fibrils from the secondary cell wall to protrude from the fiber surfaces.

The extent to which a paper product is made with refined fibers can be measured by various techniques. One type of testing for refined fibers is referred to as freeness testing. In 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9995 9995 9995 99

## 11

application. In certain applications it may be desirable to provide a creped paper product from a heavier basis weight web of fibers compared with another application. In the case of masking tape, the basis weight of the web of fibers can be at least about 10 lbs./3000 ft<sup>2</sup> so that the tape can pull off the roll and be applied without tearing as a result of hand manipulation. Of course, the basis weight could be lower depending on the care the person is willing to exercise or the tolerance the person is willing to entertain relative to tearing of the tape. In general, it is expected that masking tape can be prepared from a web of fibers having a basis weight of about 15 lbs./3000 ft<sup>2</sup> to about 40 lbs./3000 ft<sup>2</sup>, and can have a basis weight of about 20 lbs./3000 ft<sup>2</sup> to about 35 lbs./3000 ft<sup>2</sup>. For other products such as carpet seaming tape, it may be desirable to provide the creped paper product from a web of fibers having a basis weight of up to about 90 lbs./3000 ft<sup>2</sup>. Accordingly, a general range for selecting the basis weight of the web of fibers is about 10 lbs./3000 ft<sup>2</sup> to about 90 lbs./3000 ft<sup>2</sup>. The finished creped paper product refers to the creped web of fibers with additives from both wet end chemistry and size press chemistry but before latex treatment. In general, any weight of paper may be used in accordance with the present invention. Therefore, the finished creped paper product is made in weights desired by end users. However, using a paper substrate that is heavier than necessary for a particular application may not be economically efficient. In an embodiment, the finished creped paper product can include less than about 35.0 lbs./3000 ft<sup>2</sup> of paper. Paper that is too low in weight may not be suitable for use as tape. In an embodiment, the finished creped paper product can have greater than about 18.0 lbs./3000 ft<sup>2</sup> of paper. The finished creped paper product of the invention can be in the range of about 20.0 to 25.0 lbs./3000 ft<sup>2</sup> of paper.

The present invention may be better understood with reference to the following example. This example is intended to be representative of specific embodiments of the invention, and is not intended as limiting the scope of the invention.

## EXAMPLE

## Effect of Synthetic Fiber Amounts on Dry Tear Strength

Creped paper products were made by combining various percentages of polyester fiber with natural fibers and following the process described with respect to FIG. 1. The polyester fibers used can be characterized as high tenacity, 3 denier filament, 0.25 inch length fibers from Minifiber, Inc. Some of the creped paper products were impregnated with ACRONAL S 504 (an aqueous styrene/acrylic copolymer latex) available from BASF Corporation, Ontario Canada. After the creped paper products were manufactured, their dry tear strength was tested with a ProTear Electronic Elmendorf Tearing Tester, Model 60-2200, from Thwing-Albert Instrument Company. The dry tear strength was measured in accordance with TAPPI Standard T414. The results are shown in Table 1.

TABLE 1

|                   | Percentage of Synthetic Fibers | CD Tear Strength (gf) | MD Tear Strength (gf) |
|-------------------|--------------------------------|-----------------------|-----------------------|
| No Latex          | 0.0                            | 73.3                  | 53.2                  |
|                   | 3.0                            | 80.9                  | 65.5                  |
| Latex Impregnated | 0.0                            | 39.2                  | 29.3                  |
|                   | 3.0                            | 49.6                  | 41.95                 |

The results show that inclusion of 3.0% synthetic fibers increased dry tear strength for a creped paper product that has not been impregnated with latex by approximately 10.3% in

## 12

the cross direction and about 23.1% in the machine direction. The results show that inclusion of 3.0% synthetic fibers increased dry tear strength for a latex impregnated creped paper substrate by approximately 26.5% in the cross direction and approximately 43.2% in the machine direction.

The above specification provides a complete description of the manufacture and use of the composition of the invention. Since many embodiments of the invention can be made without departing from the spirit and scope of the invention, the invention resides in the claims hereinafter appended.

We claim:

1. A creped paper product comprising:

a creped paper substrate comprising a web of fibers comprising about 2 wt. % to about 5 wt. % polyester fibers based on the total weight of the fibers and about 90 wt. % to about 99.5 wt. % cellulosic fibers based on the total weight of the fibers, the creped paper substrate having a stretch of at least 3% in the machine direction according to TAPPI test T494 and a dry tear strength in the machine direction according to TAPPI test T494 at least 30% greater than an otherwise identical creped paper substrate that does not contain the polyester fibers, wherein the creped paper substrate is creped as a result of creping using a creping blade, and wherein the creped paper substrate has been treated with a latex composition so that the latex composition enters into the web of fibers; a release layer provided on a first surface of the creped paper substrate;

adhesive provided on a second surface of the creped paper substrate; and

wherein the creped paper product is provided in the form of a roll.

2. A creped paper product of claim 1, wherein the creped paper product has a dry tear strength in the machine direction according to TAPPI test T414 at least 20% greater than an otherwise identical creped paper product that does not contain the polyester fibers.

3. A creped paper product according to claim 1, wherein the creped paper product has a dry tear strength in the cross direction according to TAPPI test T414 at least 5% greater than an otherwise identical creped paper product that does not contain the polyester fibers.

4. A creped paper product of claim 1, wherein the polyester fibers have an average length of about 1 mm to about 100 mm.

5. A creped paper product of claim 1, wherein the polyester fibers have an average length of about 1 mm to about 8 mm.

6. A creped paper product of claim 1, wherein the web of fibers has a weight of about 10 lbs./3,000 ft<sup>2</sup> to 90 lbs./3,000 ft<sup>2</sup>.

7. A creped paper product of claim 1, wherein the web of fibers has a Canadian Standard Freeness value of between about 100 cm<sup>3</sup> and 850 cm<sup>3</sup> according to TAPPI test T 227.

8. A creped paper product of claim 1, comprising about 5 to about 100 crepe lines per lineal inch.

9. A creped paper product of claim 1, comprising about 20 to about 30 crepe lines per lineal inch.

10. A creped paper product according to claim 1, wherein the creped paper product comprises greater than 100 to about 200 crepe lines per lineal inch.

11. A creped paper product according to claim 1, wherein the creped paper substrate is impregnated with the latex composition.

12. A method for forming a creped paper product comprising:

creping a web of fibers comprising about 2 wt. % to about 5 wt. % polyester fibers based on the total weight of the fibers and about 90 wt. % to about 99.5 wt. % cellulosic

**13**

fibers based on the total weight of the fibers to provide a creped paper substrate having a stretch of at least 3% in the machine direction according to TAPPI test T494 and a dry tear strength in the machine direction according to TAPPI test T494 at least 30% greater than an otherwise identical creped paper substrate that does not contain the polyester fibers, wherein creping comprises creping using a creping blade;

treating the creped paper substrate with a latex composition so that the latex composition enters into the web of fibers;

providing a release layer on a first surface of the creped paper substrate;

providing an adhesive on a second surface of the creped paper substrate; and

rolling the creped paper product into the form of a roll.

**13.** A method according to claim 12, wherein the creped paper product has a dry tear strength in the machine direction according to TAPPI test T414 at least 20% greater than an otherwise identical creped paper product that does not contain the polyester fibers.

**14.** A method according to claim 12, wherein the creped paper product has a dry tear strength in the cross direction

**14**

according to TAPPI test T414 at least 5% greater than an otherwise identical creped paper product that does not contain the polyester fibers.

**15.** A method according to claim 12, wherein the polyester fibers have an average length of about 1 mm to about 100 mm.

**16.** A method according to claim 12, wherein the polyester fibers have an average length of about 1 mm to about 8 mm.

**17.** A method according to claim 12, wherein the web of fibers has a weight of about 10 lbs./3,000 ft.<sup>2</sup> to 90 lbs./3,000 ft.<sup>2</sup>

**18.** A method according to claim 12, wherein the web of fibers has a Canadian Standard Freeness value of between about 100 cm<sup>3</sup> and 850 cm<sup>3</sup> according to TAPPI test T 227.

**19.** A method according to claim 12, comprising about 5 to 15 about 100 crepe lines per lineal inch.

**20.** A method according to claim 12, comprising about 20 to about 30 crepe lines per lineal inch.

**21.** A method according to claim 5, wherein the creped paper product comprises greater than 100 to about 200 crepe lines per lineal inch.

**22.** A method according to claim 12, wherein the creped paper substrate is impregnated with the latex composition.

\* \* \* \* \*